

(No Model.)

E. WHEELER.

COMPOSITE INGOT FOR PRODUCING SEAMLESS TUBES.

No. 368,175.

Patented Aug. 9, 1887.



Fig. 9.



Fig. 10.



Witnesses.

Frank L. Emery

John F. C. Prinster

Inventor:

E. bridge Wheeler

by Leroy G. Gregory attys

# UNITED STATES PATENT OFFICE.

ELBRIDGE WHEELER, OF BOSTON, MASSACHUSETTS, ASSIGNOR TO WARE  
B. GAY, GEORGE W. GOGIN, AND HIMSELF, TRUSTEES, ALL OF SAME  
PLACE.

## COMPOSITE INGOT FOR PRODUCING SEAMLESS TUBES.

SPECIFICATION forming part of Letters Patent No. 368,175, dated August 9, 1887.

Application filed September 14, 1886. Serial No. 213,517. (No model.)

*To all whom it may concern:*

Be it known that I, ELBRIDGE WHEELER, of Boston, county of Suffolk, and State of Massachusetts, have invented an Improvement in 5 a Composite Ingot for Producing Seamless Hollow Metal Tubes, of which the following description, in connection with the accompanying drawings, is a specification, like letters on the drawings representing like parts.  
10 This invention has for its object to produce a seamless metal tube in a novel manner.  
In accordance with my invention, I first form a metal ingot by casting steel or other ductile or malleable metal—such as brass and 15 copper and their alloys—about a core composed of a center of non-metallic or silicious material, contained, for the best results, in a wooden or other combustible case or jacket, which may be enveloped by a covering of sheet 20 metal, the said combustible case or jacket when consumed forming a layer of carbon between the said center and the cast metal. The case or jacket referred to, containing the non-metallic or silicious core, and preferably enveloped by a metal covering, will, for the best 25 results, be set upon pieces of metal slabs or plates within a mold, and when so placed the metal to form the ingot will be cast into the said mold, so as to extend beyond the ends of 30 the core. The ingot thus formed will be reduced in usual manner by rolling or otherwise to form a tube of the desired diameter, and after being so reduced the said tube will be 35 cut up into desired lengths and the core removed.

Figure 1, in sectional elevation, shows one form of mold with which to practice my invention; Fig. 2, a longitudinal section of an ingot produced in the said mold in accordance 40 with my invention; Fig. 3, a section of Fig. 2 on line  $xx$ ; Fig. 4, a section through the core in Fig. 1 on line  $yy$ ; Fig. 5, a longitudinal section of a tube produced from the ingot shown in Fig. 2; Fig. 6, an end view of Fig. 45 5; Figs. 7 and 8 sectional views of modified forms of cases or jackets; Fig. 9, a longitudinal section of a tube with the core removed, and Fig. 10 an end view of Fig. 9.

The mold A, resting upon a suitable base,

A', may be of any desired construction or 5c form.

Within the mold A, I have placed a core, B, which, as herein shown, rests upon slabs or metal plates a. The core B is composed of a central portion, b, of sand or any other non-metallic or silicious material, which, for the best results, is contained in a case or jacket, b', (see Fig. 4,) of wood, paper, or other combustible material, the said case or jacket being preferably enveloped by a metallic covering, b<sup>2</sup>, of sheet-iron.

The metal cast into the mold A to surround the core B and to extend beyond its ends may be steel, copper, or brass or their alloys, or any other ductile or malleable metal which 65 when cast into the mold will heat the metal cover b<sup>2</sup> to such degree as to carbonize the layer b' of wood or other combustible material, thus producing a layer of carbon between the non-metallic or silicious center and the cast 7c metallic envelope. The ingot thus formed and composed of a center, b, of sand or other non-metallic or silicious substance, and an outer enveloping body, c, of cast metal, and an intervening layer, b', of carbon, may be reduced in usual manner, by rolling or otherwise, 75 preferably into blooms or billets. The blooms or billets so formed may be reduced to form a filled tube of the desired diameter, as shown in Figs. 5 and 6, and composed of metal c, a 80 non-metallic center, b, and an intervening layer, b', of carbon.

Referring to Fig. 7, I have shown in section a modification of my invention, wherein the non-metallic or silicious material b is contained 85 in a case or jacket, d, which is surrounded by a larger case or jacket, d', between which and the case or jacket d is placed a layer or body, b', of non-gritty non-fusible refractory material—such as German clay, plumbago, soapstone, diatomaceous earth, fossil meal, &c., either one or two or more combined, or the said layer or body may be of carbon.

Fig. 8 shows a modification wherein the case or jacket to contain the silicious or other non-metallic portion of the core is composed of a molded non-gritty and non-fusible material, or of a non-metallic compressible material of

a higher fusing point than the material to be contained in the said case or jacket.

This jacket or case may, for instance, be made from plumbago made as a crucible.

5 The layer *b'* of carbon or of non-gritty or non-fusible material mentioned, either in their dry state in a jacket or molded as described, and which is interposed between the non-metallic or silicious center and the enveloping cast metal *c*, prevents the said non-metallic or silicious center from fusing with the metal *c* cast into the mold, so that when desired the said center may be easily removed without difficulty and without damage to the boring-  
15 tool.

I do not desire to limit my invention to the particular materials herein mentioned to prevent fusion between the non-metallic or silicious core and the cast metal, as other non-com-  
20 bustible substances might be used equally well, such, for instance, as asbestos, talc, &c.

I do not herein broadly claim an ingot containing a sand core, nor do I broadly claim the employment of a sand core in an enveloping  
25 metal case or jacket, as the same is contained in my application, Serial No. 190,871, filed February 4, 1886.

I claim—

1. As an improved article of manufacture, an ingot from which to produce seamless hollow metal tubes, it comprehending a non-metallic or silicious center and a layer or body of non-gritty non-fusible material, substantially as described, surrounding the said center, and a cast-metal envelope inclosing the 35 said center and intervening body of non-gritty material, substantially as and for the purpose specified.

2. As an improved article of manufacture, an ingot from which to produce seamless hollow metal tubes, it comprehending a non-metallic or silicious center and a layer or body of carbon or other non-combustible material, an enveloping cast metal inclosing the said center, and an intervening body of carbon or 40 other non-combustible material, substantially as described.

In testimony whereof I have signed my name to this specification in the presence of two sub-  
scribing witnesses.

ELBRIDGE WHEELER.

Witnesses:

G. W. GREGORY,  
JAS. H. CHURCHILL.